

April 21, 1953

G. H. ROHRBACK ET AL.  
CORROSION INHIBITING COMPOSITION CONTAINING  
ARSENIOUS OXIDE AND POTASSIUM HYDROXIDE

Filed Dec. 22, 1951

2,635,999

2 SHEETS—SHEET 1



FIG. 1

INVENTORS  
GILSON H. ROHRBACK  
DWITE M. MCLOUD  
WILLARD R. SCOTT JR.

BY A. L. Brown  
Frank E. Johnston  
ATTORNEYS

April 21, 1953

G. H. ROHRBACK ET AL  
CORROSION INHIBITING COMPOSITION CONTAINING  
ARSENIC OXIDE AND POTASSIUM HYDROXIDE

Filed Dec. 22, 1951

2,635,999

2 SHEETS—SHEET 2



FIG. 2

INVENTORS  
GILSON H. ROHRBACK  
DWITE M. McCLOUD  
WILLARD R. SCOTT Jr.

BY A. L. Simon  
Frank C. Johnson  
ATTORNEYS

## UNITED STATES PATENT OFFICE

2,635,999

CORROSION INHIBITING COMPOSITION  
CONTAINING ARSENOSUS OXIDE AND  
POTASSIUM HYDROXIDE

Gilson H. Rohrback, Whittier, Dwite M. McCloud,  
Buena Park, and Willard R. Scott, Jr., Alham-  
bra, Calif., assignors to California Research  
Corporation, San Francisco, Calif., a corpora-  
tion of Delaware

Application December 22, 1951, Serial No. 262,994

13 Claims. (Cl. 252—8.55)

1

This invention relates to a corrosion inhibitor for use in inhibiting the corrosion of ferrous metal piping and tubing in producing wells and in pipe lines transporting crude oil. More particularly, it relates to a solid arsenous corrosion inhibitor.

The corrosion of ferrous metal tubing and piping in producing oil wells and in pipe lines transporting crude oil is now and has for some years been a serious operating problem confronting the petroleum producer. Corrosion of tubing and piping necessitates frequent interruptions of production to pull corroded tubing and piping from the well and replace them with new material. The essential features of a corrosive environment very commonly encountered in producing oil wells, and one in which the corrosion inhibitor of this invention is highly effective, include a ferrous metal in contact with oil, brine, and gas containing carbon dioxide, gas liquid interfaces in contact with the metal, and areas of turbulent liquid flow in contact with the metal surfaces. The metal in this environment is corroded away by direct attack of carbonic acid which is greatly accelerated by electrochemical phenomena arising out of the contact of the phase interfaces with the metal and out of the contact of turbulent flowing liquid with the metal surface. Substantially all of the acidity of the production stream stems from the presence of carbon dioxide. The acidity is quite low, the pH not being lower than 3 and being ordinarily in the range 4 to 6. When a ferrous metal is exposed to the production effluent under quiescent conditions where there is no movement of the liquid or of free gas bubbles through the liquid, the corrosion rate observed is usually less than about 25% of that observed under actual producing conditions which include turbulent motion of the liquid in contact with the metal and the presence of minute gas bubbles which contact the metal. In laboratory apparatus in which the separate influence of the three corrosive factors was studied, i. e., direct acid attack, electrochemical attack attributable to turbulent liquid flow, and electrochemical attack attributable to the presence of finely-divided gas bubbles which contact the metal surfaces, it was found that the relative rate of corrosion due to direct acid attack was 4 units, and that the relative rate of corrosion when either the condition of liquid turbulence or finely-divided gas bubbles moving through the liquid was superimposed on the presence of the acid medium, the relative corrosion rate immediately increased to 14 units. From these observations it is clear that the corrosion problem would not be solved by the employment of an inhibitor which would eliminate only the corrosive action due to direct acid attack and that the corrosion problem here pre-

2

sented can be solved only if the additional electrochemical corrosion attributable largely to physical conditions is markedly reduced. The corrosion inhibitor of this invention is especially well adapted to minimizing the corrosion of ferrous metals in the environment and by the mechanisms described.

A variety of physical setups is found in producing oil wells which determine the manner of introduction of the corrosion inhibitor into the well. Some wells have open annuli and a corrosion inhibiting solution can be lubricated into the well through the open annulus. Some wells have packed-off annuli and the corrosion inhibitor must be introduced through the production tubing by pumping an inhibitor solution to the well bottom and permitting it to flow upward with the production stream or by dropping a solid corrosion inhibitor through the tubing to the well bottom and producing the well. In condensate wells, where there is no liquid production stream, the corrosion inhibitor to be effective must in some manner be applied to the interior surface of the tubing without the aid of a liquid production stream to carry and spread it.

A solid corrosion inhibitor which can be placed at or near the well bottom by dropping it through the well tubing can be utilized effectively in all types of wells if the solid inhibitor has the following properties: First, it must be an effective inhibitor at low concentrations. Only relatively small amounts of an inhibitor can be introduced into a well by dropping the solid inhibitor through the tubing. Some commonly used inhibiting chemicals such as dichromates and caustic soda will inhibit satisfactorily if used in large amounts, but these materials are not suitable for injection into the well in solid form since the maintenance of the desired concentration requires very frequent interruption of the production for the introduction of further amounts of the inhibitor. A suitable chemical inhibitor for injection into the well through the tubing in solid form would be one that provides protection against corrosion at concentrations of about one to five parts per million in the produced water. Second, an effective solid corrosion inhibitor should have a high persistency in its inhibiting effect. To be practical, the injections of a solid inhibitor should not be made more often than once in twenty-four hours, and preferably once in several days, or once a week. High persistency of the inhibitor or inhibiting film formed on the metal surfaces of the tubing is highly desirable in solid inhibitor injection. Third, a successful solid corrosion inhibitor should be highly soluble in well water. This is particularly desirable if the inhibitor is to be used in a condensate well. Relatively insoluble or highly insoluble materials could easily cause plugging of the tubing.

Fourth, a solid corrosion inhibitor should have a high density so that the solid inhibitor will fall through the production stream while the well is being produced. If the solid inhibitor has this property, the production need be interrupted for only the few minutes necessary to introduce the solid into the tubing. Fifth, the solid inhibitor, if it is to be effective in a condensate well, should soften at or slightly below the temperature existing at the zone of condensation. Condensate wells produce little or no formation water and much of a water-soluble chemical that falls below the condensate zone will not be returned with the production. If the solid inhibitor softens or melts at temperatures from about 150 to 200° F., the solid will be spread on the hot tubing wall as it falls in the well.

Arsenous compounds, particularly the alkali metal arsenites or slurries of arsenous oxide with alkali metal hydroxides and water, meet the above-described requirements with respect to effectiveness at low concentration, persistence, and solubility admirably. Particular arsenous compositions hereinafter described meet not only the first three requirements, but also the require-

4  
hydroxide in the composition when the water content is approximately constant. The compositions are designated soft when they are readily molded by manual pressure.

The properties of arsenous oxide-potassium hydroxide-water mixtures were further studied to determine the range of compositions which produced hard products at atmospheric temperature.

10 From these studies it was determined that the ratio by weight of arsenous oxide to potassium hydroxide in compositions having softening points above 100° F. lie in the range from 1.8:1 to 5:1 and that the water content should be from 1 to 3.0 parts by weight to each 15 parts by weight of arsenous oxide and potassium hydroxide together. Compositions having softening points above 150° F. must contain  $As_2O_3$  and KOH at weight ratios in the range 2:1 to 4.25:1 and compositions having higher softening points especially useful when placed at the bottom of average producing wells where high temperatures exist should have  $As_2O_3$  to KOH weight ratios in the range from 2.25:1 to 3.0:1. Representative observations are set out in the following Table II.

Table II

|                                |      |      |      |       |      |      |       |       |       |
|--------------------------------|------|------|------|-------|------|------|-------|-------|-------|
| As <sub>2</sub> O <sub>3</sub> | 8.6  | 9.57 | 9.57 | 10.05 | 10.5 | 10.5 | 11.45 | 11.45 | 12.37 |
| Parts KOH                      | 6.4  | 5.43 | 5.43 | 4.95  | 4.5  | 4.5  | 3.55  | 3.55  | 2.63  |
| Water                          | 1.61 | 1.28 | 1.6  | 1.6   | 1.26 | 1.68 | 1.25  | 1.56  | 1.24  |
| Ease of Mixing                 | Good | Good | Good | Good  | Good | Good | Good  | Good  | Good  |
| Set Consistency                | Soft | Soft | Hard | Hard  | Hard | Hard | Hard  | Hard  | Hard  |
| Softening Temp., °F.           |      | 150  | 280  | 280   | 280  | 280  | 235   | 235   | 160   |

ments with respect to density and to softening point in a remarkable manner.

It has now been found that a hard, dense homogeneous solid corrosion inhibitor can be prepared by intimately mixing arsenous oxide, potassium hydroxide and water and cooling the resultant mixture to remove exothermic heat of reaction. The mixture contains from 1 to 3.0 parts by weight of water to 15 parts by weight of potassium hydroxide and arsenous oxide together and the ratio of arsenous oxide to potassium hydroxide in the mixture is in the range 1.8:1 to 5:1. An organic hydroxy compound such as ethylene glycol and other similar materials set forth hereinafter is desirably substituted for part of the water in the composition.

Compositions containing these ingredients in these proportions are very hard at ordinary temperatures, have a high density above about 3.0 g. per cubic centimeter and are thermoplastic in the sense that they become soft at temperatures from about 150 to about 280° F., and finally become liquid at higher temperatures.

Numerous compositions consisting essentially of arsenous oxide, potassium hydroxide and water were prepared and their properties at atmospheric temperature were examined. The composition and properties of several of these mixtures are summarized in Table I

Table I

|                              |      |      |      |      |
|------------------------------|------|------|------|------|
| Parts by weight $As_2O_3$    | 6    | 8    | 10   | 12.5 |
| Parts by weight KOH          | 9    | 7    | 5    | 2.5  |
| Parts by weight, Water added | 0.4  | 1.1  | 1.25 | 1.63 |
| Parts by weight, Total water | 2.0  | 2.0  | 2.0  | 2.0  |
| Base of Mixing**             | Fair | Good | Good | Good |
| Set Consistency              | Soft | Soft | Hard | Soft |

\*Pelleted commercial KOH containing 15% by weight of  $H_2O$ .

\*\*Refers only to consistency of mixture, not to speed of setting.

From the data in the above table it is clear that room temperature hardness is clearly related to the ratio of arsenous oxide to potassium

35 From the table it is clear that the character of the compositions changes abruptly when the arsenous oxide to potassium hydroxide ratio goes above about 1.75:1 and that the softening temperature falls off as the ratio approaches 5:1. The softening temperature of the solid  $As_2O_3$ -KOH- $H_2O$  compositions is effected not only by the ratio of arsenous oxide to potassium hydroxide, but also by the amount of water contained in the composition. In general, the compositions soften at lower temperatures as the water content of the composition rises. The minimum water content for practical purposes is 1 part by weight of water to 15 parts by weight of arsenous oxide and potassium hydroxide together. When it is attempted to employ smaller amounts of water, it is extremely difficult to make a homogeneous mixture of the three components before the partially mixed materials set. If more than 3.0 parts by weight of water to 15 parts by weight of arsenous oxide and potassium hydroxide combined are employed, the compositions are definitely soft at 100° F. and remain soft or liquid at that temperature. Compositions having softening points above 150° F. should contain no more than 2.5 parts by weight of water for each 15 parts by weight of arsenous oxide and potassium hydroxide together and should contain at least 1 part by weight of water to each 15 parts by weight of arsenous oxide and potassium hydroxide together to permit adequate mixing before setting occurs. Compositions having higher softening points above 200° F. which are especially useful when placed at the bottom of producing wells where high temperatures prevail should contain not more than 2.25 parts by weight of water for each 15 parts by weight of arsenous oxide and potassium hydroxide together. The effect of varying the water content of the compositions is illustrated by Figure 1 of the drawings, which is a graphical representation of the variation of softening temperature with

water content when varying amounts of water are added to 15 parts by weight of arsenous oxide and potassium hydroxide. The ratio of arsenous oxide to potassium hydroxide in the experiments providing the data for the construction of Figure 1 was 2.33:1.

From Figure 1 it is evident that the softening point of the compositions can be varied from 150° F. to 290° F. by varying the water content. For example, a solid inhibitor composition having a softening point of about 280° F. would be best suited for use in the high pressure flowing wells of Louisiana, where bottom hole temperatures may be as high as 260° F., whereas a solid inhibitor composition softening at about 180° F. would be well suited for use in the condensate wells of West Texas. In the condensate wells it is desirable that the solid inhibitor soften suffi-

forms suitable for introduction into the well. The substitution of ethylene glycol for a part of the water in the inhibitor compositions also increases the resistance of the solid product to shearing and impact forces. When water alone is used, the solid tends to be somewhat grainy and brittle and, when it is cast in stick form, the stick may be rather readily broken by shearing or impact forces. This characteristic is undesirable if it is intended to drop the solid inhibitor in stick form into the well tubing. The sticks strike against the tubing as they fall and may be broken into small pieces which are carried up by the production stream before reaching the well bottom.

The compositions of several solid inhibitors in which varying amounts of water were replaced by ethylene glycol are shown in Table III.

Table III

|                                                      |                 |                 |                 |                 |
|------------------------------------------------------|-----------------|-----------------|-----------------|-----------------|
| Parts by weight As <sub>2</sub> O <sub>3</sub> ..... | 10.5.....       | 10.5.....       | 10.5.....       | 10.5.....       |
| Parts by weight KOH.....                             | 4.5.....        | 4.5.....        | 4.5.....        | 4.5.....        |
| Parts by weight H <sub>2</sub> O.....                | 1.68.....       | 1.26.....       | 1.47.....       | 1.68.....       |
| Parts by weight Ethylene Glycol.....                 | .63.....        | 1.26.....       | 1.05.....       | 0.84.....       |
| Parts by weight Total Liquid.....                    | 2.31.....       | 2.52.....       | 2.52.....       | 2.52.....       |
| Ease of Mixing.....                                  | Good.....       | Fair.....       | Good.....       | Good.....       |
| Pourable after Complete Mixing.....                  | Yes.....        | Yes.....        | Yes.....        | Yes.....        |
| Softening Temperature.....                           | 270-290° F..... | 270-290° F..... | 270-290° F..... | 270-290° F..... |

ciently in the tube so that the inhibitor will rub off on the hot tubing as the solid falls in the well.

The softening point of the solid



compositions may also be regulated, though less reliably, by substituting sodium hydroxide for a small part of the potassium hydroxide. From 0.1% to 5% by weight of the potassium hydroxide may be replaced by sodium hydroxide and the softening point of the composition is lowered. When sodium hydroxide is used to regulate the softening point, care must be exercised that the amount be kept small since it exercises extraordinary effects on the softening point, so much in fact that when



and



mixtures, each of which would set hard at atmospheric temperature, are combined before setting, the combined mixture remains permanently liquid.

The solid As<sub>2</sub>O<sub>3</sub>—KOH·H<sub>2</sub>O inhibitor compositions above described may be improved in two respects by substituting an organic hydroxy compound such as ethylene glycol for a part of the water. The substitution of these materials for part of the water very considerably reduces the rate at which the compositions set up as hard solids when the three ingredients are mixed. When arsenous oxide, potassium hydroxide and water are mixed in the proportions above described, they tend to set very rapidly. This characteristic gives rise to a serious problem in commercial production of the inhibitor compositions where it is desirable to mix large batches of the inhibitor and pour the mixture into molds to set. The setting is so rapid that the compositions set up as solids in the mixing vessel before pouring can be completed. The substitution of ethylene glycol for part of the water greatly reduces the setting rate and thus facilitates commercial production of the solid inhibitor cast in

All of the compositions shown in the table were readily pourable after complete mixing and no difficulty was experienced in making the mixture and pouring it from the mixing vessel to casting molds without solidification occurring in the mixing vessel. The resultant sticks were much less brittle and more difficult to fracture than were corresponding compositions in which all of the liquid was water. The softening temperatures of the compositions are not adversely affected by the substitution of the ethylene glycol. If appreciable improvement in the solid is to be achieved, at least 10% by weight of water should be replaced by ethylene glycol and usually 20 to 50% of the water is replaced by ethylene glycol where greater durability and slower setting time are desired. The preferred organic hydroxy compound for use in the inhibitor compositions is ethylene glycol. However, it has been determined that other organic hydroxy compounds will perform the same function, for example, aliphatic alcohols containing up to 12 carbon atoms per molecule, diethylene glycol and triethylene glycol produce similar effects on the setting time and resistance to fracture of the inhibitor compositions.

The inhibitor compositions above described are desirably cast in the form of pellets or sticks. The most usual form is a cylindrical stick from 1 to 3 feet in length and from 1 to 2 inches in diameter, that is, a diameter generally adapted to permit the fall of the stick through conventional well tubing. The sticks ordinarily weigh from 1 to 10 pounds and have a density above about 3 g. per cubic centimeter. Their mass and density are such that they readily fall through the production stream of the average producing well so that the production need be interrupted only for the few minutes which are required to introduce the stick into the well tubing. The introduction of such a stick every three to ten days will ordinarily bring the corrosion rate of a well down to an acceptable low level and maintain it there.

Since the arsenical compounds are poisonous, the sticks are desirably wrapped or coated with some non-toxic material in the interest of safe

handling. The wrapping or coating may be either functional or non-functional and may be an integral part of the stick as it is dropped into the well, or may be removable at the time of injection.

When the well to be treated is a flowing well discharging a production stream of oil, brine and carbon dioxide, a metal having a standard oxidation reduction potential above 0.5 and below 2.5 volts, such as magnesium, aluminum, zinc, and their alloys, forms an excellent functional integral coating for the inhibitor. Corrosion inhibiting cartridges can be prepared by pouring the molten corrosion inhibitor into a thin walled (0.01 to 0.05 inch) metal tube or cylinder and permitting it to solidify there. The ends of the tube or top of the cylinder are then closed. The closure can be made by capping with a metallic cap, or crimping the tubing, or sealing with a high melting point wax or asphalt. The metallic coating is an integral part of the inhibitor cartridge as it is dropped into the well. The metal casing prevents the solid inhibitor stick from being broken during its fall through the tubing, and the metal is functional in its action in the well and not merely a container for the inhibitor. Magnesium, for example, slowly dissolves in dilute carbonic acid contained in the well water and, in dissolving, neutralizes part of the acid; in addition, metals such as magnesium, zinc, aluminum and their alloys provide cathodic protection against electrolytic corrosion.

Other integral coatings which are non-functional may be employed such as a high melting point wax or an oil-soluble or water-soluble plastic material. The solidified inhibitor stick can be dipped in these materials and allowed to dry and the surface film of these materials provides protection to personnel against handling hazards. In the well the protective coating is rapidly dissolved, placing the inhibitor composition in contact with the production stream.

The inhibitor sticks may also be protected by an outer container which is removed prior to the introduction of the inhibitor stick into the well. The hot, soft corrosion inhibitor is poured into paper cylinders and allowed to solidify there. The paper tubing is peeled away from the stick before dropping it into the well tubing. It has been found that if the hot corrosion inhibitor mixture is poured into untreated paper tubes, some difficulty is experienced in attempting to remove the paper from the hardened stick. However, if the paper is greased with a fairly heavy grease, or covered with a water-impervious coating such as shellac or plastic, prior to the introduction of the molten inhibitor composition into the paper tube, the paper may easily be removed from the solidified stick. Alternatively, the molten inhibitor can be poured into a rubber cylinder and allowed to solidify there. When the inhibitor is solid, the top of the rubber cylinder is pressed together and sealed with rubber cement.

The corrosion inhibitors of this invention have been tested in flowing wells discharging oil, brine and carbon dioxide and have reduced the corrosion rate, as determined by the iron count of the produced water, from 75 to 90%.

The corrosion inhibitors of the invention have also been tested in condensate wells and found effective. The results of one such test are graphically illustrated in Figure 2 of the drawings. This well was a Louisiana condensate well. Prior to initiation of the test this well was being re-

ularly treated with commercially available organic corrosion inhibitor sticks which are rather widely used. The effectiveness of the corrosion inhibitors to inhibit corrosion of ferrous metal tubing was determined by observing the iron count of produced water before and after treatment. The iron count, a measure of the corrosion rate, is the number of parts per million of iron calculated as ferric oxide contained in the produced water as determined by the thiocyanate colorimetric method (Scott's Standard Method of Chemical Analysis, 5th Edition, Van Nostrand, 1939, page 486). From Figure 2 it will be seen that the inhibitor of the invention was markedly superior to an inhibitor currently in commercial use, even when used in very much smaller quantities.

We claim:

1. A hard, dense solid comprising an intimate mixture of arsenous oxide, potassium hydroxide and water, the ratio by weight of arsenous oxide to potassium hydroxide being in the range from 1.8:1 to 5:1 and the water content being at least one part by weight and not more than about 3.0 parts by weight to each 15 parts by weight of arsenous oxide plus potassium hydroxide.
2. A hard, dense solid consisting essentially of a reaction product of arsenous oxide, potassium hydroxide and water, the proportions of the reactants being such that the ratio by weight of  $\text{As}_2\text{O}_3$  to KOH is in the range from 2:1 to 4.25:1 and that from 1 to about 3.0 parts by weight of water are present for each 15 parts by weight of arsenous oxide plus potassium hydroxide.
3. A hard, dense solid consisting essentially of a reaction product of arsenous oxide, potassium hydroxide and water, the proportions of the reactants being such that the ratio by weight of  $\text{As}_2\text{O}_3$  to KOH is in the range 2:1 to 4.25:1 and that from 1.0 to 2.25 parts by weight of water are present for each 15 parts by weight of arsenous oxide plus potassium hydroxide.
4. A hard, dense solid formed by intimately mixing 15 parts by weight of arsenous oxide and potassium hydroxide with 1 to 3.0 parts by weight of water and ethylene glycol, the ratio of arsenous oxide to potassium hydroxide being in the range 1.8:1 to 5:1 and the ratio of water to ethylene being in excess of 1 to 1.
5. A hard, dense solid formed by mixing 10 to 12.5 parts by weight of arsenous oxide, 2.5 to 5 parts by weight of potassium hydroxide and 1 to about 3.0 parts by weight of water, the arsenous oxide and potassium hydroxide totaling 15 parts by weight.
6. A hard, dense solid formed by mixing 10 to 12 parts by weight of arsenous oxide, 3 to 5 parts by weight of potassium hydroxide and 1 to about 3.0 parts by weight of water, the arsenous oxide and potassium hydroxide totaling 15 parts by weight.
7. A hard, dense solid formed by mixing 10 to 12.5 parts by weight of arsenous oxide, 2.5 to 5 parts by weight of potassium hydroxide and 1 to 3.0 parts by weight of a mixture of water and ethylene glycol.
8. The composition as defined in claim 7, wherein the mixture of ethylene glycol and water contains about 10% by weight of ethylene glycol.
9. The method as defined in claim 7, wherein the mixture of ethylene glycol and water contains from 10 to 50% by weight of ethylene glycol.
10. A hard, dense solid containing 10 to 12 parts by weight of arsenous oxide, 3 to 5 parts

by weight of potassium hydroxide and 1.0 to about 3.0 parts by weight of a mixture of water and ethylene glycol.

11. The composition as defined in claim 10, wherein the mixture of water and ethylene glycol contains 10 to 50% by weight of ethylene glycol.

12. The method of inhibiting corrosion in a producing oil well delivering a production stream comprising petroleum, brine and carbon dioxide gas which comprises periodically interrupting the production, dropping a solid corrosion inhibitor formed by intimately mixing arsenous oxide, potassium hydroxide and water, the ratio by weight of arsenous oxide to potassium hydroxide in the mixture being in the range from 1.8:1 to 5:1 and the water content of the mixture being at least one part by weight and not more than about three parts by weight to each fifteen parts by weight of arsenous oxide plus potassium hydroxide, through the well tubing to 20 the bottom of the well and producing the well.

13. A composition as defined in claim 4, wherein the content of water and ethylene glycol is in the range from 1 to 2.5 parts by weight.

5

GILSON H. ROHRBACK.  
DWITE M. McCLOUD.  
WILLARD R. SCOTT, JR.

## References Cited in the file of this patent

## UNITED STATES PATENTS

| Number    | Name         | Date           |
|-----------|--------------|----------------|
| 1,638,710 | Sherbino     | Aug. 9, 1927   |
| 1,877,504 | Grebe et al. | Sept. 13, 1932 |

## OTHER REFERENCES

J. Mellor—"Comprehensive Treatise on Inorganic and Theoretical Chemistry"—vol. IX—1929, page 117.